

United States Patent [19]  
Ingersoll

[11] 3,929,474  
[45] Dec. 30, 1975

[54] TARNISH RESISTANT SILVER BASED  
DENTAL CASTING ALLOY CAPABLE OF  
BONDING TO PORCELAIN

[75] Inventor: Clyde E. Ingersoll, Tonawanda,  
N.Y.

[73] Assignee: Williams Gold Refining Company  
Incorporated, Buffalo, N.Y.

[22] Filed: Aug. 5, 1974

[21] Appl. No.: 494,566

[52] U.S. Cl. .... 75/172 G; 75/173 R

[51] Int. Cl.<sup>2</sup> .... C22C 5/04; C22C 5/06

[58] Field of Search ..... 75/173 R, 172 G

[56] References Cited

UNITED STATES PATENTS

1,229,037 6/1917 Cooper ..... 75/173 R  
1,999,866 4/1935 Capillon et al. ..... 75/172 G

2,070,271 2/1937 Gwyn ..... 75/173 R X  
2,222,544 11/1940 Spanner ..... 75/173 R X  
3,155,467 11/1964 Yamamoto et al. ..... 75/173 R X

FOREIGN PATENTS OR APPLICATIONS

628,572 4/1936 Germany ..... 75/173 R

Primary Examiner—L. Dewayne Rutledge

Assistant Examiner—E. L. Weise

Attorney, Agent, or Firm—Christel & Bean

[57]

ABSTRACT

An alloy composition comprising about 35-60% Pd, at least about 0.5-7% of one member of the group consisting of Cr, Fe, In and Sn and from about 0 to 5% of the group consisting of Si, Ni, Co, Ta, and Ti, and the rest Ag, has been found useful in the dental arts where a porcelain is required to be fused directly to the alloy.

7 Claims, No Drawings

## TARNISH RESISTANT SILVER-BASED DENTAL CASTING ALLOY CAPABLE OF BONDING TO PORCELAIN

Reference is made to U.S. patent application Ser. No. 494,565 filed of even date by the instant inventor relating to silver-based alloys useful in the dental and jewelry arts.

### BACKGROUND OF THE INVENTION

#### 1. Field of the invention

This invention relates to silver-palladium alloys employed in the dental and jewelry arts which are resistant to tarnishing; have superior ductility and work hardening characteristics and have a coefficient of thermal expansion close to that of porcelain, and can form an oxide coating so that the alloy may be fire bonded to porcelain.

#### 2. Description of the Prior Art

The American Dental Association (ADA) has had Specification 5 for many years, which included four types of casting alloys in common use in dentistry. Type IV, of greater significance here, relates to alloys for having a 150 minimum Vickers hardness and hardneable to 220 minimum Vickers hardness, which are for use in partial dentures, bars, clasps, and unit castings. In addition to the four types, ADA has a proposed specification for alloys having high melting temperature and high yield strength (similar to Type IV), and a coefficient of thermal expansion close to that of the porcelain to be fired to it and which forms an oxide coating for bonding to the porcelain.

### SUMMARY OF THE INVENTION

The present invention comprises alloys of silver and palladium containing at least one member of the class consisting of Cr, Fe, In and Sn and optionally containing one or more members of the class consisting of Si, Ni, Co, Ta, and Ti. Such alloys have good tarnish resistance, ductility and work hardening characteristics, have coefficients of thermal expansion close to that of porcelain, and can be directly bonded thereto and have Vickers hardness values of from 150 to above 220.

### OBJECTS OF THE INVENTION

It is an object of this invention to provide a silver based alloy for bonding directly to porcelain.

It is a further object of the invention to provide a silver based alloy having the requisite properties of ductility, hardness, work hardening, tarnish resistance and coefficient of thermal expansion for use in the dental arts for bonding directly to porcelain, together with the properties necessary for casting, such as fluidity for filling a mold completely and for polishing.

Further objects of the invention will become apparent from the following description and claims.

### DESCRIPTION OF THE INVENTION

A dental alloy meeting the requirements of the ADA proposed specification set forth above should have in addition to the hardness requirements, good tarnish resistance and good work hardening characteristics.

Ductility is a highly desirable property in dental alloys since, in many instances, the dentist must burnish the dental piece for better adaptation. Brittle margins are likely to break off during such burnishing operations.

Good work hardening characteristics are important for easier manipulation by the dentist or technician. Dental alloys are usually supplied in the form of wrought pieces. If the alloy work hardens rapidly, only a small amount of reduction can be achieved after each strain relief treatment.

### TARNISH RESISTANCE

Publication No. 31,008 of the Department of Commerce (dated Sept. 23, 1927) gives the results of tests on the tarnishability of silver-based alloys. In the publication, the alloys were exposed to sodium polysulfide for a period of eight minutes and the discolorations noted. In the present case, this test was modified by substituting ammonium sulfide, which was found to give more reproducible results. In the corrosion tests employed, cast bar specimens were prepared by first grinding and polishing by normal metallurgical methods followed by sandblasting the surface to be exposed to ammonium sulfide for eight minutes.

A numerical scale was established by exposing pure silver bars to ammonium sulfide for times ranging from 0 to 145 seconds, giving a scale of 0 for no exposure to 10, almost black. In making the test, a portion of the test bar was covered so that the exposed portion and unexposed portion could be directly compared. Dental amalgam rated 9 on this scale, an alloy of 75 silver-25 palladium rated 5. An ADA certified gold alloy rated between 0 and 1 and was assigned  $\frac{1}{2}$ . To be acceptable for dental work of the type covered in ADA Specification 5, and the proposed specification the tarnish rating should be no higher than about 5.5.

### HARDNESS

Since the hardness is not translatable from one alloy system to another, some other mechanical property must be employed to compare different systems. In the present case, the 0.1% offset yield strength was used as the comparable property. The Vickers hardness shown in the table is for a silver base alloy of this invention having the same 0.1% offset yield strength as the ADA Specification 5 Type alloy.

TABLE I

| Type<br>(ADA SPEC.<br>NO. 5) | 0.1% Offset Yield Strength<br>(Gold<br>or Silver Base Alloy) | Vickers Hardness<br>(Silver Base<br>Alloy) |
|------------------------------|--------------------------------------------------------------|--------------------------------------------|
| IV                           | 44,500+                                                      | 200+                                       |

These values are all in the "as cast" condition.

While copper has been employed as a hardening agent for silver-palladium alloys (see U.S. Pat. No. 2,198,400), too high a concentration of copper is known to cause brittleness (see U.S. Pat. No. 2,259,668). As shown in copending case Ser. No. 494,565, a number of elements may be added to silver-palladium alloys to increase the Vicker hardness numbers. It has been found that in order to meet the requirements of proposed ADA Specification and to have suitable tarnishing resistance and cold reduction properties, the additional alloying elements should be at least the member from the group selected from the class of Cr, Fe, In and Sn and, optionally, one or more members of the group selected from Si, Ni, Co, Ta and Ti. The alloys of this invention comprise about 28-64% Ag, about 34-60% Pd, about 0.5-7% of at least one member of the class consisting of Cr, Fe, In or Sn and

0 to about 5% of Si, Ni, Co, Ta or Ti.

### THERMAL EXPANSION

Because of the high coefficients of thermal expansion imparted by In and Sn, the amounts of these elements which may be employed in the alloys of the invention is less than the upper limit of 10% in the alloys of my copending application, Ser. No. 494,565. Zn is unusable as an additive in the present case because of its high vapor pressure at porcelain firing temperatures.

The following table gives a number of examples of alloys exemplary of the present invention.

| Alloy No. | EXAMPLE (ELEMENTS GIVEN IN %) |      |    |    |     |     |        |     | Cold Reduction |     |
|-----------|-------------------------------|------|----|----|-----|-----|--------|-----|----------------|-----|
|           | Ag                            | Pd   | Cr | Fe | In  | Sn  | Other  | HV  |                |     |
| 1         | Bal                           | 57.7 | —  | —  | 1   | 6   | Si 0.7 | 215 | 3              | 68% |
| 2         | Bal                           | 50.4 | —  | —  | 1   | 1   | Ni 5.0 | 216 | 4              | 62% |
| 3         | Bal                           | 45   | 2  | —  | —   | —   | Co 2.0 | 217 | 4              | 80% |
| 4         | Bal                           | 45.9 | —  | 4  | —   | —   | Ta 0.5 | 212 | 4              | 89% |
| 5         | Bal                           | 46.5 | —  | 2  | —   | —   | Ni 2.0 | 212 | 2              | 90% |
| 6         | Bal                           | 48   | —  | 5  | 0.5 | 0.5 |        | 221 | 3              | 86% |
| 7         | Bal                           | 37.5 | 5  | —  | 0.5 | 0.5 | Ti 1.0 | 210 | 3              | 81% |

What is claimed is:

1. An alloy consisting essentially of about 28-64% AG, about 37.5-57.7 % Pd, about 0.5-7% of at least one member of the class consisting of Cr, Fe, In and Sn and from 0 to about 5% of a member of the class consisting of Si, Ni, Co, Ta, Ti, all totalling 100%; said alloy having a Vickers hardness of 150-220; said alloy when containing Sn further containing a member selected from the group consisting of about 0.5% in, 1.0% Ti, 5.0% Ni, 17% Si, and 5% Fe; and said alloy when con-

taining Fe further containing a member selected from the group consisting of about 0.5% Ta, about 2.0% Ni, and about 0.5% In and about 0.5% Sn.

2. The alloy of claim 1 wherein the composition is about 37.5% Pd, about 0.5% In, about 0.5% Sn, about 1% Ti and the balance Ag.

3. The alloy of claim 1 consisting essentially of about 48% Pd, about 5% Fe, about 0.5% In, about 0.5% Sn, and the balance Ag.

10 4. The alloy of claim 1 consisting essentially of about 46.5% Pd, about 2% Fe, about 2% Ni and the balance Ag.

25 5. The alloy of claim 1 consisting essentially of about 45.9% Pd, about 4% Fe, about 0.5% Ta and the balance Ag.

6. The alloy of claim 1 consisting essentially of about 45% Pd, about 2% Cr, about 2% Co and the balance 30 Ag.

7. The alloy of claim 1 consisting essentially of about 57.7% Pd, about 1% In, about 1% Sn, about 5% Ni, and the balance Ag.

\* \* \* \* \*

35

40

45

50

55

60

65